

## UNITED STATES PATENT OFFICE.

JOSEPH A. SMITH, OF ATTLEBORO, MASSACHUSETTS.

## PLATED ARTICLE AND ITS MANUFACTURE.

No Drawing.

Application filed January 23, 1925. Serial No. 4,271.

*To all whom it may concern:*

Be it known that I, JOSEPH A. SMITH, a citizen of the United States, residing at Attleboro, in the county of Bristol and 5 State of Massachusetts, have invented certain new and useful Improvements in Plated Articles and Their Manufacture, of which the following is a specification.

My invention relates to improvements in 10 plated articles and an improved method of their manufacture.

My invention particularly relates to the process of tight coating or inter-alloying a metal article, usually a steel article, with a 15 layer of a metal of substantially low melting point. I am aware that it is old to electro-deposit a thin layer of zinc and on subjecting the electro-plated article to heat to tight coat the zinc to the metal. I am also 20 aware that it is old to electro-deposit a layer of a metal of a substantially low melting point such as cadmium to a metal article and by subjecting the article to heat to inter-alloy the cadmium with the article to 25 form a protective coating. The disadvantages of either of these processes have been 30 as follows: In the heating treatment a large amount of the electro-deposited layer of zinc or cadmium is oxidized off, thereby necessi- 35 tating the use of a large amount of electro-deposited metal and consequent loss of metal. As an inter-alloying takes place be- 40 tween the outer electro-deposited layer and the metal of the article there is always a certain amount of iron or steel or other base 45 metal employed drawn to the surface in the inter-alloying and so the article becomes not completely rustproof as often claimed.

In my process I electro-deposit or other- 50 wise coat on the metal article an intermediate layer of a metal of a substantially low melting point such as zinc, tin, silver, cad- 55 mium or other suitable metal or alloy and electro-deposit or otherwise coat on the sur- 60 face of the intermediate layer a layer of a metal of a higher melting point than that of the intermediate layer and I then subject 65 the coated article to heat under conditions causing an alloying of the intermediate 70 layer and the metal of the article. It is a 75 matter of common knowledge that when

electro-plated articles are heated to the required degree the electro-deposited metal, crystalline when laid, forms a sheet or tight coating of metal over the metal article. As 55 in my process I preferably only heat the article to an amount below the melting point of the intermediate layer, the outer protective layer usually remains crystalline as electro-deposited. The preferably thinner 60 outer layer however, prevents the intermediate layer from being oxidized off as it becomes inter-alloyed with the metal of the article, thus effecting a great saving in metal. As no substantial amount of inter- 65 alloying takes place between the outer layer and the intermediate layer or the metal of the article, it is obvious that none of the base metal will be drawn to the outer surface and that the article is more rust-proof than 70 any hitherto constructed.

These and such other objects of my invention as may hereinafter appear will be best understood from a description of the specific method about to be described illustrat- 75 ing an embodiment of my invention.

The article to be plated which may comprise a musical instrument wire, a spring or any other suitable metal article herein called the base metal article is cleaned and polished 80 in the usual manner to prepare for the electro-deposition of the plating process by cleaning it of all rust and dirt preferably with a very fine grade of emery cloth. If necessary it may also be cleaned by dipping 85 it in a dilute sulfuric acid or other chemical solution and finally in water.

The next step in the process consists in coating on the base metal an intermediate layer of a metal of a substantially low melt- 90 ing point which is preferably accomplished by an electro-plating bath of the following composition: Chloride of zinc 4 ozs., cyanide of potassium 4 ozs., sal-ammoniac 2 ozs. to each gallon of water. A sufficient deposit 95 of this solution may be obtained in five minutes with a voltage of six, though a heavier deposit may be laid thereon if desired by plating for a longer period.

The article is then preferably rinsed in 100 water and then coated with a layer of a metal of a substantially higher melting

point preferably by electro-plating a layer of nickel thereon. A suitable electro-plating bath for this purpose is double nickel salts 8 ozs., single nickel salts 2 ozs., boracic acid 1 oz. to each gallon of water. A sufficient coating may be obtained in about five minutes with a voltage of 2½.

The article is then preferably dipped into a yellow ochre solution which tends to prevent the formation of heat spots during the heating treatment, though this step may be dispensed with if thought advisable.

The article is then heated in a furnace or a gas flame preferably at a temperature of substantially 600° F. for an appreciable length of time varying from five minutes to four hours to cause an inter-alloying of the intermediate layer with the base metal of the article and to change the intermediate layer from a crystalline structure into a sheet. The outer preferably thinner nickel layer is not appreciably affected by the heat treatment at this temperature and may remain as a protective layer. Even though the protective crystalline nickel layer may become worn in use there will remain a tight coated intermediate zinc layer underneath very resistant to wear. The furnace may be heated up to 600° F., the article inserted and taken out when the temperature again rises to 600° F. to give an inter-alloying suitable for most purposes. After removal from the furnace, the ochre solution is washed off and the article buffed and polished.

As stated in place of zinc other metals of a substantially low melting point such as cadmium, silver, tin or other suitable metals or alloys may be employed. In place of nickel as the outer protective layer, gold, silver, copper or other suitable alloys or metals may be employed.

It is obvious that by this process I have provided a metal article having all the advantages of an article having a coating alloyed thereto and the advantages of having an outer coating of metal of a higher melting point.

It is understood that my invention is not limited to the specific processes or articles described and that various deviations may be made therefrom without departing from the spirit and scope of the appended claims.

What I claim as new and desire to secure as Letters Patent is:

1. The process of coating metal articles, which comprises coating the article with an intermediate layer of a metal of a substantially low melting point, in coating the intermediate layer with a layer of a metal of a substantially higher melting point and then subjecting the coated article to heat under conditions causing an alloying of the intermediate layer and the metal of the article without any substantial inter-alloying with the outer layer.

2. The process of coating metal articles, which comprises electro-depositing on the article an intermediate layer of a metal of a substantially low melting point, in electro-depositing on the intermediate layer a layer of a metal of a substantially higher melting point and then subjecting the coated article to heat under conditions causing an alloying of the intermediate layer and the metal of the article without any substantial inter-alloying with the outer layer.

3. The process of coating metal articles which comprises coating the article with an intermediate layer of zinc, in coating the zinc layer with a layer of nickel and then subjecting the coated article to heat under conditions causing an alloying of the zinc and the metal of the article without any substantial inter-alloying with the nickel layer.

4. The process of coating metal articles which comprises electro-depositing on the article an intermediate layer of zinc, electro-depositing on the zinc layer a layer of nickel and then subjecting the coated article to heat under conditions causing an alloying of the zinc layer and the metal of the article without any substantial inter-alloying with the nickel layer.

5. The process of coating metal articles, which comprises coating the article with an intermediate layer of a metal of a substantially low melting point, in coating the intermediate layer with a layer of a metal of a substantially higher melting point and then subjecting the coated article to a heat somewhat less than the melting point of the metal of the intermediate coated layer for a substantial period of time to cause an alloying of the intermediate layer and the metal of the article.

6. The process of coating metal articles which comprises electro-depositing on the article an intermediate layer of metal of a substantially low melting point, in electro-depositing on the intermediate layer a layer of a metal of a substantially higher melting point and then subjecting the coated article to a heat somewhat less than the melting point of the metal of the intermediate coated layer for a substantial period of time to cause an alloying of the intermediate layer and the metal of the article.

7. The process of coating metal articles which comprises coating the article with an intermediate layer of zinc, in coating on the zinc layer a layer of nickel and then subjecting the coated article to a heat of substantially 600° F. from five minutes to four hours to cause an alloying of the zinc and the metal of the article.

8. The process of coating metal articles which comprises electro-depositing on the article an intermediate layer of zinc, in electro-depositing on the zinc layer a layer of nickel and then subjecting the coated article to a

heat of substantially 600° F. from five minutes to four hours to cause an alloying of the zinc layer and the metal of the article.

9. A metal article having a coating of a metal of a substantially low melting point alloyed thereto and a coating of a metal of a substantially higher melting point thereon.

10. A metal article having a coating of a metal of substantially low melting point al-

loyed thereto and an electro-deposited layer <sup>10</sup> of a metal of a substantially higher melting point thereon.

11. A metal article having a coating of zinc alloyed thereto and a coating of nickel <sup>15</sup> thereon.

In testimony whereof I affix my signature.

JOSEPH A. SMITH.